

1

3,170,793

### PHOTOGRAPHIC FIXING BATH

Marilyn Levy, Red Bank, N.J., assignor to the United States of America as represented by the Secretary of the Army

No Drawing. Filed Oct. 27, 1960, Ser. No. 65,549

2 Claims. (Cl. 96—61)

(Granted under Title 35, U.S. Code (1952), sec. 266)

The invention described herein may be manufactured and used by or for the Government for governmental purposes, without the payment of any royalty thereon.

This invention relates to photographic processing and particularly to the fixing of photosensitive materials after the image has been developed therein.

In the photographic system wherein silver halide emulsions are used as the sensitive medium after development the residual unexposed halide must be completely removed. This is accomplished by bathing in a solution of sodium thiosulphate until all of the halide is removed. To insure that this operation is complete and to protect the delicate wetted emulsion certain other ingredients may be added, for example, a small quantity of acid such as acetic acid neutralizes the alkali carried by the emulsion from the developer. A hardener also is added such as potassium alum and a preservative such as sodium sulphite.

In the use of such fixing baths the undeveloped silver halide grains are dissolved and removed from the emulsion. Since thiosulphate ions convert to the silver thiosulphate complex in a fixing bath, the activity of the bath becomes diminished with constant use. The formulation of sodium iodide as a result of the conversion of silver iodide to silver thiosulfate complex also reduces the rate of fixation. If the bath is used too long it may lose its ability to remove all of the unused silver salts from the emulsion. These unused salts in time will decompose and stain the negative or print.

This progressive consumption of activity of the fixing bath has many disadvantages. It may lead to unstable and inferior end results due to the difficulty in determining when to discard the bath or it may result in setting up a safety factor which requires discarding the bath before its useful activity is consumed.

The invention adds an ingredient to the fixing bath which controls the bath activity and prolongs the life of the bath. By so doing the quantity of chemicals consumed is reduced. The practice of this invention also provides means for maintaining quality control of the end products which has not heretofore been readily achievable.

By adding a suitable quantity of colloidal silica to the fixing bath its active life will be greatly prolonged. The silica which is thoroughly dispersed in the bath acts to neutralize the deterrent effect of accumulated silver salts in the bath. Thus the bath continues to function for a long period after the same bath without the additive would have ceased to be effective.

Since the colloidal silica immediately becomes effective in the presence of dissolved silver salts its corrective function maintains full activity of the fixing bath thruout the processing of large quantities of sensitive materials.

Processing with the bath of the invention insures consistent high quality results as well as greatly extended area

2

of sensitive material processed compared with conventional fixing baths. Colloidal silica as an additive has been found to be particularly successful in increasing the capacity of fixing baths and has the added property of being chemically neutral to the other bath ingredients. The silica functions only to absorb and otherwise render the accumulated salts in the bath ineffective in slowing the fixing potential of the bath.

The invention in its broad aspect includes fixing baths having any desired composition of chemicals including sodium thiosulphate as the main dissolving agent for the undeveloped silver halide in the sensitive emulsion. The hypo may be used alone or with various proportions of control chemicals such as acetic acid, sodium sulphite and a hardener such as potassium alum.

Into the above suggested compositions a quantity of colloidal silica is dispersed to constitute the formulation of the invention.

An example of a formulation embodying the invention is as follows:

|                                                 |       |      |
|-------------------------------------------------|-------|------|
| Water                                           | liter | 1.0  |
| Sodium thiosulphate                             | grams | 240  |
| Sodium sulphite                                 | do    | 15   |
| Acetic acid 28%                                 | cc    | 48   |
| Potassium alum                                  | grams | 15   |
| Colloidal silica dispersed in above composition | do    | 1-15 |

The above composition or a similar one including the proper amount of colloidal silica is used after the film or print has been exposed, developed and desirably immersed in an acidic stop bath. The developed material is immersed in the fixing bath for the usual time of from 10 to 20 minutes for films and 5 to 10 minutes for prints. During such immersion the conventional degree of agitation should be carried out. The processed material is then washed and dried in the usual manner.

It has been found that in the bath of the invention an accurate and consistent determination may be made of its total fixing capacity either by trial or in some other manner. Subsequent fixing operations can then be based upon this determination. Knowing their potentiality the baths may be used up to their full capacity without fear of forcing them beyond the safety point. This means that full benefit may be derived from the added fixing capacity which the invention imparts to the bath.

A further feature of the invention is its adaptation to baths having increased viscosity which is a valuable attribute under certain environmental conditions. For example there are military operations which require that photographic processing to be carried out in flight or in moving vehicles where vibration and erratic bodily movements of solution containers disrupt open tray operations. It has been found that solutions of increased viscosity may successfully be used under such conditions.

The properties of the present invention may readily be extended to include such increased viscosity solutions. If the addition of a normal amount of silica suffices to extend the capacity of the bath fails to produce the required viscosity more silica may be added until the required immobility of the solution is achieved. The bath having the added silica will also function with the required effectiveness to extend the fixing capacity thereof.

What is claimed is:

1. A fixing bath comprising the following ingredients:

|                                               |       |           |
|-----------------------------------------------|-------|-----------|
| Water                                         | liter | 1         |
| Sodium thiosulphate                           | grams | 50 to 300 |
| Sodium sulphite (desiccated)                  | do    | 5 to 30   |
| Acetic acid 28%                               | cc    | 10 to 100 |
| Potassium alum                                | grams | 5 to 30   |
| Boric acid crystals                           | do    | 3 to 15   |
| Colloidal silica dispersed in the<br>solution | do    | 5 to 300  |

2. A fixing bath comprising an aqueous solution of sodium thiosulphate in the proportion of 50 to 300 grams per liter of water, a quantity of preservative, a quantity of gelatine hardening agent, an acidifying agent in quantity to change the pH value of the bath less than 5%, the

15

quantity of preservative and hardening agent having a total weight less than  $\frac{1}{3}$  to  $\frac{1}{4}$  of the weight of sodium thiosulphate and a quantity of colloidal silica in an amount from 20 to 250 grams per liter.

References Cited by the Examiner

UNITED STATES PATENTS

|           |       |        |         |
|-----------|-------|--------|---------|
| 2,616,807 | 11/52 | Land   | 96-61 X |
| 2,871,121 | 1/59  | Kimura | 96-61   |

OTHER REFERENCES

Photo Lab Index, Section 2, page 17, Quarterly Supplement No. 50 (New Page), Morgan and Lester, New York.

NORMAN G. TORCHIN, Primary Examiner.

MILTON STERMAN, LOUIS P. QUAST, Examiners.